# EUROPEAN PATENT SPECIFICATION

(11) **EP 3 323 924 B1**
(45) Date of publication and mention of the grant of the patent: **22.12.2021**
(21) Application number: 17193076.1
(22) Date of filing: 26.09.2017
(51) Int. Cl.: D04H 1/4218, D04H 1/4226, D04H 1/587, D04H 1/60, F16L 59/02

(54) **METHOD FOR MANUFACTURING A DOUBLE OR MULTI-LAYER MINERAL WOOL INSULATION**
VERFAHREN ZUR HERSTELLUNG EINER ZWEI- ODER MEHRSCHICHTIGEN ISOLIERUNG AUS MINERALWOLLE
PROCÉDÉ DE FABRICATION D'UNE ISOLATION EN LAINE MINÉRALE À DEUX OU PLUSIEURS COUCHES

(30) Priority: 16.11.2016 FI 20165860
(43) Date of publication of application: 23.05.2018
(73) Proprietor: Paroc Group Oy, 00180 Helsinki (FI)
(72) Inventor: Mattila, Hannu-Petteri, 21280 Raisio (FI); Honkasalo, Mika, 21600 Parainen (FI); Lundström, Kim, 21600 Parainen (FI)
(74) Representative: Sole, Timo

(56) References cited:
- EP-A1- 1 180 182
- EP-A2- 1 571 247
- WO-A1-2008/034951
- JP-A- 2003 082 567
- US-A- 5 093 069
- US-A- 5 778 492

## Description

The present invention relates to a method for manufacturing a double or multi-layer mineral wool insulation. The invention further relates to a mineral wool insulation manufactured by the method.

Various methods for manufacturing a multilayer insulation of mineral wool are known from prior art. WO2014090670 presents a method, in which is formed a base layer of mineral wool, in which the fibres are substantially perpendicular in relation to the main surfaces of the base layer, which is cured. On top of the cured base layer is spread an uncured mineral wool layer, and the combination is taken into a curing oven, in which the surface layer is compressed at least 50%. EP1180182 presents a method, in which a thin mineral wool sheet is cut from a mineral wool mat with a horizontal cutting blade, the cut sheet being compressed between the rollers into a denser form and spread back onto the rest of the mineral wool mat, from which the sheet was cut. Finally, loose material forming a rigid surface layer is spread onto the top surface of the compressed mineral wool layer and the product obtained is coated with a thin polyester fabric and taken to a curing treatment. The object is to produce a very rigid surface layer, the density of which is at least 450 kg/m³. EP 1 180 182 discloses a mineral fibre insulating product comprising a mineral fibre insulating layer and at least one rigid surface layer, said surface layer comprising mineral material bound together by a binding agent.

The object of the present invention is to provide a relatively simple and easily implemented method for manufacturing a double or multi-layer mineral wool insulation utilizing recycling material, which is obtained either from the same facility, in which the mineral wool products are manufactured, or from customers as surplus material returns.

To achieve this object, a method according to the invention is characterized in that, in the method, on a mineral wool manufacturing line is continuously produced a mineral wool mat having a bottom side and a top side defining the main surfaces of the mineral wool mat, the fibres of which are located substantially in levels parallel with said main surfaces, that, in the method, onto at least one of said main surfaces is brought an additional insulation layer containing recycled material, which contains crushed and/or pulverized mineral wool and into which recycled material is mixed binding agent in a powdered form before it is brought onto said at least one main surface of the mineral wool mat, that, in the method, the layer of recycled material is compressed into a mat-like layer to a desired density wherein the degree of compression is 50% or more, before it is brought onto said at least one main surface of the mineral wool mat, and that, finally, the mineral wool insulation formed from the mineral wool mat and the additional insulation layer of recycled material added onto its at least one main surface is taken to a curing treatment.

In a method according to the invention it is possible, if needed, to further compress the mineral wool insulation formed from the mineral wool mat and the additional insulation layer comprising recycled material before or in the curing oven in order to achieve a desired density (which can also be the final density).

The layer of recycled material is formed as different in at least one of its properties in comparison to the mineral wool mat layer, the property being selected from a group including fibre chemistry, fibre length, fibre orientation, binding agent, density, layer thickness, compression strength. In the method, onto the outer surface of the additional insulation layer of recycled material is preferably added a coating layer of fibreglass fabric before the mineral wool insulation is taken to the curing treatment. In the method, an additional insulation layer containing recycled material is preferably brought onto both main surfaces of the mineral wool mat. In a preferred further embodiment of the method, a second mineral wool mat is brought onto the other side of the additional insulation layer containing recycled material brought onto one main surface of the mineral wool mat, wherein the additional insulation layer of recycled material forms the middle layer of the mineral wool insulation.

The advantage of the present invention is that there is no need to make major changes to an existing mineral wool mat manufacturing line in order to introduce the method according to the invention. The mineral wool mat is manufactured normally and it does not require special handling before the additional layer is fed onto at least one main surface of the mineral wool mat. The additional layer is fed, for example, between the belt conveyors as compressed to the desired density onto the mineral wool mat and the insulation product thus obtained is taken to a curing treatment, for example, into a curing oven, in which the binding agents in the mineral wool mat and the additional insulation layer harden under the influence of heat and the layers simultaneously adhere to each other.

In the following, the invention is described in more detail with reference to the accompanying drawings, in which:
- Fig. 1: shows a preferred embodiment of an apparatus suitable for performing a method according to the invention, and
- Fig. 2: shows a diagrammatic cross-section of a mineral wool insulation manufactured by the method.

Insulation products of mineral wool, such as, for example, a raw mineral wool mat used in the manufacture of mineral wool boards and in the form of a mat, is manufactured on a basic production line by first forming mineral wool fibres from molten rock, from which, through pleating a primary mat of mineral wool, a secondary mat of mineral wool is formed. This manner of producing so-called raw wool is described, for example, in WO 94/16162, WO 2006/070055 and WO 03/008353.

In an apparatus according to Fig. 1, at the starting end (not shown) of a manufacturing line, a mineral wool mat 2 of raw wool manufactured in a per se known manner is transported between the belt conveyors 4, 5 as compressed to a desired density and further by means of the rollers 9 towards the curing oven 8. The apparatus includes a feeding apparatus attached to the manufacturing line of the mineral wool mat 2, the feeding apparatus including the belt conveyors 6, 7, between which the additional insulation layer 3 is compressed to a desired density before it is fed onto the top surface 11 of the mineral wool mat 2. The degree of compression is 50% or more depending on the desired density. The mat-like additional insulation layer 3 is pressed by the guide roller 10 against the top surface of the mineral wool mat. The apparatus preferably includes means for feeding an optional coating material 13 from a roll 14 onto the outer surface of the additional insulation layer in order to keep the fibre material and the binding agent of the additional insulation layer in place in the additional insulation layer in the air flow of the curing oven. As the coating material 13 is preferably used fibreglass fabric or felt. Preferably, onto both sides of the mineral wool mat 2 are added additional insulation layers 3, 3' and also onto both outer surfaces of the additional insulation layer is preferably added a coating material 13.

Fig. 2 shows as a cross-section a mineral wool insulation 1 manufactured by the method according to the invention, the mineral wool insulation having a middle layer of mineral wool mat 2 and the additional insulation layers 3, 3' formed from recycled material on both of its sides. The amount of recycled material is preferably approx. 16% of the amount of the mineral wool mat. The middle layer 2 formed from a mineral wool mat of a mineral wool insulation 1 produced according to the invention is preferably in the range of 60-80 kg/m³ in density and its thickness is, for example, 100 mm. The density of the additional insulation layer 3, 3' formed from recycled material is preferably in the range of 150-250 kg/m³, its thickness being, for example, in the range of 10-20 mm.

The material of the additional insulation layer is primarily shredded/pulverized/crushed mineral wool material, to which is added in connection with shredding/pulverizing/crushing or thereafter dry powder-like binding agent, which can be different than the binding agent used in the mineral wool mat. The recycled material can also contain other crushed/chopped materials, such as concrete/wood fractions or fire retardants or other additives. Examples of additives acting as fire retardants are plaster, slaked lime, calcium carbonate, calcium sulphate hemihydrate, dolomite, aluminium hydroxide, aluminium sulphate, magnesium hydroxide, magnesium carbonate, montmorillonite, bentonite. Examples of additives acting as fire retardants expanding at high temperatures are vermiculite, perlite, pumice, and expanding varieties of clay.

By varying the thickness and density of the layers they can, if desired, be rendered to have different properties, such as, for example, compression strength.

## Claims

1. A method for manufacturing a double or multi-layer mineral wool insulation (1), wherein on a mineral wool manufacturing line is continuously produced a mineral wool mat (2) having a bottom side and a top side defining the main surfaces of the mineral wool mat, the fibres of which are located substantially in levels parallel with said main surfaces, wherein onto at least one of said main surfaces is brought an additional insulation layer (3, 3') containing recycled material, which contains shredded and/or crushed and/or pulverized mineral wool, wherein into the recycled material is mixed binding agent in a powdered form before it is brought onto said at least one main surface of the mineral wool mat (2), **characterized in that**, in the method, the layer (3, 3') of recycled material is compressed into a mat-like layer to a desired density wherein the degree of compression is 50% or more, before it is brought onto said at least one main surface of the mineral wool mat, and that, finally, the mineral wool insulation (1) formed from a mineral wool mat (2) and an additional insulation layer of recycled material (3, 3') added onto its at least one main surface is taken to a curing treatment (8).

2. A method according to claim 1, **characterized in**
**that**, in the method, the layer (3, 3') of recycled material is formed as different in at least one of its properties in comparison to the mineral wool mat layer (2), the property being selected from a group containing fibre chemistry, fibre length, fibre orientation, binding agent, density, layer thickness, compression strength.

3. A method according to any one of claims 1-2, **characterized in**
**that**, in the method, onto the outer surface of the additional insulation layer (3, 3') of recycled material is added a coating layer (13) of fibreglass fabric before the mineral wool insulation (1) is taken to the curing treatment.

4. A method according to any one of claims 1-3, **characterized in**
**that**, in the method, an additional insulation layer (3, 3') containing recycled material is brought onto both main surfaces of the mineral wool mat (2).

5. A method according to any one of the preceding claims, **characterized in**
**that**, in the method, the density of the mineral wool mat coming from the line is 60-80 kg/m³ and the surface layer of recycled material is compressed to a density of 150-250 kg/m³.

6. A method according to any one of the preceding claims, **characterized in**
**that**, in the method, the thickness of the mineral wool mat coming from the line is 80-120 mm, preferably approximately 100 mm, and the thickness of the surface layer is in the range of 10-20 mm.

7. A method according to any one of the preceding claims, **characterized in**
**that**, in the method, the portion of recycled material in the final product is in the range of 10-18%, preferably approx. 14-16%.

## Patentansprüche

1. Verfahren zur Herstellung einer doppel- oder mehrschichtigen Mineralwolledämmung (1), wobei in einer Anlage zur Herstellung von Mineralwolle kontinuierlich eine Mineralwollmatte (2) hergestellt wird, die eine Unterseite und eine Oberseite hat, die die Hauptflächen der Mineralwollematte festlegen, deren Fasern im Wesentlichen in Ebenen parallel zu den Hauptflächen liegen, wobei auf mindestens eine der Hauptflächen eine zusätzliche Dämmschicht (3, 3') aufgebracht ist, die recyceltes Material enthält, welches geschredderte und/oder zerkleinerte und/oder pulverisierte Mineralwolle enthält, wobei in das recycelte Material ein Bindemittel in einer pulverisierten Form eingemischt wird, bevor es auf die mindestens eine Hauptfläche der Mineralwollematte (2) aufgebracht wird, **dadurch gekennzeichnet,**
**dass** bei dem Verfahren die Schicht (3, 3') von recyceltem Material zu einer mattenähnlichen Schicht mit einer gewünschten Dichte komprimiert wird, wobei der Kompressionsgrad 50 % oder mehr beträgt,
bevor sie auf die mindestens eine Hauptfläche der Mineralwollematte aufgebracht wird, und dass schließlich die Mineralwolledämmung (1) aus einer Mineralwollematte (2) und einer zusätzlichen Dämmschicht aus recyceltem Material (3, 3'), auf mindestens eine Hauptfläche aufgebracht, einer Aushärtungsbehandlung (8) zugeführt wird.

2. Verfahren nach Anspruch 1, **dadurch gekennzeichnet, dass** bei dem Verfahren die Schicht (3, 3') aus recyceltem Material in mindestens einer ihrer Eigenschaften im Vergleich zur Mineralwollematte (2) unterschiedlich ausgebildet ist, wobei die Eigenschaft aus einer Gruppe ausgewählt wird, die Faserchemie, Faserlänge, Faserausrichtung, Bindemittel, Dichte, Schichtdicke, Kompressionsstärke enthält.

3. Verfahren nach Anspruch 1-2, **dadurch gekennzeichnet, dass** bei dem Verfahren auf die Außenfläche der zusätzlichen Dämmschicht (3, 3') aus recyceltem Material eine Deckschicht (13) aus Glasfasergewebe aufgebracht wird, bevor die Mineralwolledämmung (1) der Aushärtungsbehandlung zugeführt wird.

4. Verfahren nach Anspruch 1-3, **dadurch gekennzeichnet, dass** bei dem Verfahren eine zusätzliche Schicht (3, 3'), die recyceltes Material enthält, auf beide Hauptflächen der Mineralwollematte (2) aufgebracht wird.

5. Verfahren nach einem der vorhergehenden Ansprüche, **dadurch gekennzeichnet, dass** bei dem Verfahren die Dichte der Mineralwollematte, die aus der Anlage kommt, 60-80 kg/m³ beträgt, und die Oberflächenschicht des recycelten Materials ist bis zu einer Dichte von 150-250 kg/m³ komprimiert.

6. Verfahren nach einem der vorhergehenden Ansprüche, **dadurch gekennzeichnet, dass** bei dem Verfahren die Dicke der Mineralwollematte, die aus der Anlage kommt, 80-120 mm, vorzugsweise ca. 100 mm, beträgt, und die Dicke der Oberflächenschicht liegt im Bereich von 10-20 mm.

7. Verfahren nach einem der vorhergehenden Ansprüche, **dadurch gekennzeichnet, dass** bei dem Verfahren der Anteil von recyceltem Material am Endprodukt im Bereich von 10-18 %, vorzugsweise ca. 14-16 %, liegt.

## Revendications

1. Procédé de fabrication d'une isolation en laine minérale double ou multicouche (1) dans lequel, sur une chaîne de fabrication de laine minérale, est produite en continu une natte de laine minérale (2) dotée d'une face inférieure et d'une face supérieure définissant les surfaces principales de la natte en laine minérale dont les fibres se situent substantiellement à des niveaux parallèles auxdites surfaces principales, dans lequel, sur au moins une desdites surfaces principales, est posée une couche d'isolation supplémentaire (3, 3') contenant du matériau recyclé qui contient de la laine minérale déchiquetée et/ou écrasée et/ou pulvérisée, et on mélange dans le matériau recyclé de l'agent liant sous forme poudreuse avant de le mettre sur ladite au moins une surface principale de la natte en laine minérale (2), **caractérisé en ce que**,
dans le procédé, la couche (3, 3') de matériau recyclé est comprimée en une couche de type natte jusqu'à une densité désirée, le degré de compression étant de 50 % ou plus,
avant de la mettre sur ladite au moins une surface principale de la natte en laine minérale et que, finalement, l'isolation en laine minérale (1) formée d'une natte de laine minérale (2) et d'une couche d'isolation supplémentaire de matériau recyclé (3, 3') ajoutée sur son au moins une surface principale est emportée vers un traitement de durcissement (8).

2. Procédé selon la revendication 1, **caractérisé en ce que**, dans le procédé, la couche (3, 3') de matériau recyclé est formée de manière à être différente dans au moins une de ses propriétés comparativement à la couche de natte de laine minérale (2), la propriété étant sélectionnée dans un groupe contenant la chimie des fibres, la longueur des fibres, l'orientation des fibres, l'agent liant, la densité, l'épaisseur de couche, la force de compression.

3. Procédé selon l'une quelconque des revendications 1 à 2, **caractérisé en ce que**, dans le procédé, sur la surface extérieure de la couche d'isolation supplémentaire (3, 3') de matériau recyclé, on ajoute une couche de revêtement (13) en tissu à base de fibre de verre avant que l'isolation en laine minérale (1) soit emportée vers le traitement de durcissement.

4. Procédé selon l'une quelconque des revendications 1 à 3, **caractérisé en ce que**, dans le procédé, une couche d'isolation supplémentaire (3, 3') contenant du matériau recyclé est mise sur les deux surfaces principales de la natte en laine minérale (2).

5. Procédé selon l'une quelconque des revendications précédentes, **caractérisé en ce que**, dans le procédé, la densité de la natte en laine minérale provenant de la chaîne est de 60 à 80 kg/m3 et que la couche superficielle de matériau recyclé est comprimée jusqu'à une densité de 150 à 250 kg/m3.

6. Procédé selon l'une quelconque des revendications précédentes, **caractérisé en ce que**, dans le procédé, l'épaisseur de la natte de laine minérale provenant de la chaîne est de 80 à 120 mm, de préférence d'environ 100 mm, et que l'épaisseur de la couche superficielle est de l'ordre de 10 à 20 mm.

7. Procédé selon l'une quelconque des revendications précédentes, **caractérisé en ce que**, dans le procédé, la part de matériau recyclé dans le produit final est de l'ordre de 10 à 18 %, de préférence d'environ 14 à 16 %.
